

## UNITED STATES PATENT OFFICE.

JAMES A. BURTON, OF BROOKLYN, NEW YORK.

## LUBRICANT.

No Drawing.

Application filed May 25, 1922. Serial No. 563,684.

*To all whom it may concern:*

Be it known that JAMES A. BURTON, a citizen of the United States of America, residing at 421 Park Place, Brooklyn, in the 5 county of Kings and State of N. Y., has invented certain new and useful Improvements in Lubricants, of which the following is a specification.

The present invention relates to lubricants and more particularly to that class 10 of liquid lubricants adapted for use on leaf springs of motor cars, leaf springs of electric and steam railroad cars, leaf springs of wagons and the like, or more broadly to 15 lubricants for use where the rubbing of metal surfaces together is liable to cause objectionable squeaking. The lubricant is also of especial value when applied to bolts and nuts which are to be separated, particularly 20 after the same have rusted to some extent. A special object of the invention is to provide a lubricant which will readily penetrate between the leaves of springs and will loosen frozen or rusted connections and 25 avoid objectionable noises due to the rubbing of metallic surfaces against each other. Other and further objects will be obvious from the reading of this specification.

There have been many compositions proposed for application to leaf springs, for 30 preventing the same from emitting objectionable sounds, when the vehicle is operated. In many cases it was necessary to separate the leaves of the spring, by means 35 of a sharp tool, such as a chisel or screwdriver and to insert the lubricant, either in a solid or liquid condition between the leaves. This entailed considerable laborious work, and is generally not practised extensively. 40 Many of the compositions heretofore proposed have given good results for a short period, but did not permanently overcome the difficulty. With the composition of the present case, it has been demonstrated that 45 a single application of the material will overcome the objections referred to, for a considerable period.

In the preferred form of the invention I employ the materials mentioned below, preferable 50 in the proportions stated, but it will be understood that these proportions can be varied more or less, without sacrificing the entire benefits of the composition.

As a base and vehicle, I employ three 55 quarts of crude oil, preferably oil of a non-

asphaltic base, such as paraffin oil. In place of crude oil, high viscosity lubricating oil could also be employed but the same is more expensive. With the amount above stated of the heavy oil, I use 18 ounces of a refined 60 oil of relatively low viscosity, preferably kerosene. It is unadvisable to use gasoline or other highly volatile oils for this purpose, and while kerosene is to some extent volatile, it will remain sufficiently long to 65 accomplish the purpose of completely carrying the lubricant into the very fine interstices or spaces between the leaves of the spring. With the above ingredients, I also employ a mineral lubricant, preferably 70 graphite. This may be employed to the extent of six ounces, and of course should be in a finely divided condition. It may be simply ground to an impalpable powder, or deflocculated graphite could be employed. 75 For most purposes it is not necessary to use the deflocculated material which is many times more expensive than the finely powdered graphite. With the above ingredients I also employ liquids which are somewhat 80 volatile, but which are capable of greatly increasing the penetrating properties of the mixture.

Thus I may use:

7 ounces of commercial ether, 85  
3 drachms of amyl acetate,  
3 drachms of ethyl acetate,  
2 drachms of ethyl butyrate,  
5 minims of oil of cassia (oil of cinnamon). 90

These ingredients, in addition to greatly increasing the penetrating properties, and the capillary action of the product also improves its odor to considerable extent, and also imparts a lively appearance and a 95 bronzy color.

The above proportions mentioned are given by way of illustration, for the manufacture of one gallon of the oil. Obviously the quantities can be increased for commercial 100 manufacture.

The very essential characteristics of the product is its capillary action, which is very much greater than that of any similar product which I have found on the market. The 105 graphite remains in suspension persistently and does not settle out to any very great extent. Obviously the can or bottle can be shaken up, if it has been allowed to stand for a long period, say, several months, be- 110

fore making an application of the oil. The mixture will penetrate between the leaves of leaf springs, around and to the threads of rusted nuts and bolts and the like. It will spread over metallic surfaces in all directions, even vertically upwards.

The amyl acetate and ethyl acetate and ethyl butyrate above referred to can be generically described as "lower fatty acid esters 10 of the lower alkyl groups". These substances are not to be confused however, with fatty esters of high fatty acids, such as triolein, which do not have the power of increasing the capillarity of the mixture of say 15 crude oil and kerosene.

Experience has shown that when applying this material, as a single application to the leaf springs of an ordinary automobile, the objectionable squeakiness is completely 20 overcome for a period of many months, so

that frequent applications of the material are not necessary.

The amyl acetate, ethyl acetate and ethyl butyrate are to some extent the equivalents of each other and other similar low fatty 25 acid esters of low alkyl groups also can be substituted, the combination of the three specified substances seems to give rather better results than any of the others.

I claim:

A lubricant for leaf springs and the like comprising: 3 quarts of crude petroleum, 18 ounces of kerosene, 6 ounces of comminuted graphite, 7 ounces of ethyl ether, 3 drachms of amyl acetate, 3 drachms of ethyl acetate, 35 2 drachms of ethyl butyrate, 5 minims of oil of cassia.

In testimony whereof I affix my signature.

JAMES A. BURTON.

30

35